

Feb. 17, 1970

MICHIO MATSUOKA ET AL

3,496,512

NON-LINEAR RESISTORS

Filed May 10, 1967



Michio Matsuoka,  
Takeshi Masuyama and  
Yoshio Oida,

INVENTORS

BY Wenderoth, Lund & Ponack

ATTORNEYS

3,496,512

## NON-LINEAR RESISTORS

Michio Matsuoka, Nishinomiya-shi, Takeshi Masuyama, Takatsuki-shi, and Yoshiro Iida, Hirakata-shi, Japan, assignors to Matsushita Electric Industrial Co., Ltd., Osaka, Japan

Filed May 10, 1967, Ser. No. 637,492  
Claims priority, application Japan, May 16, 1966,  
41/31,594

Int. Cl. H01c 7/10, 7/04, 1/14  
U.S. Cl. 338—20

7 Claims

### ABSTRACT OF THE DISCLOSURE

New non-linear resistors having non-ohmic resistance are provided. Such resistors comprise a sintered wafer comprising, as an active ingredient, zinc oxide, and silver electrodes applied to opposite surfaces of said sintered wafer. A method is provided for making such resistors comprising applying a silver electrode paint to the opposite surfaces of the sintered wafer, heating said silver electrode paint in an oxidizing atmosphere at 100° to 850° C. so as to produce silver electrodes adhered to said surfaces and connecting lead wires to said silver electrode by a conductive connection means.

### NON-LINEAR RESISTORS

This invention relates to non-linear resistors having non-ohmic resistance and more particularly to varistors comprising zinc oxide and silver electrodes applied thereto.

Various non-linear resistors such as silicon carbide varistors, selenium or cuprous oxide rectifiers and germanium or silicon p-n junction diodes, are known. The electrical characteristics of such a non-linear resistor are expressed by the relation:

$$I = \left(\frac{V}{C}\right)^n$$

where V is the voltage across the resistor, I is the current flowing through the resistor, C is a constant equivalent to the voltage at a given current and exponent n is a numerical value greater than 1. The value of n is calculated by the following equation:

$$n = \frac{\log_{10}(I_2/I_1)}{\log_{10}(V_2/V_1)}$$

where V<sub>1</sub> and V<sub>2</sub> are the voltages at given currents I<sub>1</sub> and I<sub>2</sub>, respectively. Conveniently, I<sub>1</sub> and I<sub>2</sub> are 10 ma. and 100 ma. respectively. The desired value of C depends upon the kind of application to which the resistor is to be put. It is ordinarily desirable that the value of n be as large as possible since this exponent determines the degree to which the resistors depart from ohmic characteristics.

Silicon carbide varistors are most widely used as non-linear resistors and are manufactured by mixing fine particles of silicon carbide with water, ceramic binder and/or conductive material such as graphite or metal powder, pressing the mixture in a mold to the desired shape, and then drying and firing the pressed body in air or non-oxidizing atmosphere. Silicon carbide varistors with conductive materials are characterized by a low electric resistance, i.e. a low value of C and a low value of n whereas silicon carbide varistors without conductive materials have a high electric resistance, i.e. a high value of C and a high value of n. It has been difficult to manufacture silicon carbide varistors characterized by a high n and a low C. For example, silicon carbide varistors with graphite have been known to exhibit n values from 2.5 to 3.3 and C-values from 6 to 13 at a given current of 100 ma., and

silicon carbide varistors without graphite show n-values from 4 to 7 and C-values from 30 to 800 at a given current of 1 ma. with respect to a given size of varistor, e.g. 30 mm. in diameter and 1 mm. in thickness.

Conventional rectifiers comprising selenium or cuprous oxide have an n-value less than 3 and a C-value of 5 to 10 at a given current of 100 ma. with respect to a specimen size of 20 mm. in diameter. In this case, the thickness of sample does not affect the C-value.

A germanium or silicon p-n junction resistor has an extremely high value of n but its C-value is constant, e.g. of the order of 0.3 or 0.7 at a given current of 100 ma. because its diffusion voltage in the V-I characteristics is constant and cannot be changed remarkably. It is necessary for obtaining a desirable C-value to combine several diodes in series and/or in parallel. Another disadvantage of such diodes is their complicated steps involved in their manufacture, with resultant high cost. As a practical matter, the use of diode resistors is not widespread at the present in view of their high cost even though they may have a high value of n.

An object of this invention is to provide a non-linear resistor having a high value of n and a low value of C.

25 A further object of this invention is to provide a non-linear resistor capable of being made by a simple manufacturing method which results in a low cost.

25 A further object of this invention is to provide a non-linear resistor characterized by a high stability to temperature, humidity and electric load.

30 Another object of this invention is to provide a non-linear resistor, the C-value of which can be controlled.

35 These and other objects of the invention will become apparent upon consideration of the following description taken together with the accompanying drawing in which the single figure is a partly cross-sectional view through a non-linear resistor in accordance with the invention.

Before proceeding with a detailed description of the non-linear resistors contemplated by the invention, their construction will be described with reference to the aforesaid figure of drawing wherein reference character 10 designates, as a whole, a non-linear resistor having, as its active element, a sintered wafer 1 of electrically conductive ceramic material according to the present invention.

40 Sintered wafer 1 is prepared in a manner hereinafter set forth, and is provided with a pair of electrodes 2 and 3 having specified compositions and applied in a suitable manner hereinafter set forth, on two opposite surfaces of the wafer.

45 The wafer 1 is a sintered plate having any one of various shapes such as circular, square, rectangular, etc. Wire leads 5 and 6 are attached conductively to the electrodes 2 and 3, respectively, by a connection means 4 (solder or the like).

50 According to the present invention, sintered wafer 1 consists essentially of, as an active ingredient, zinc oxide (ZnO). It is preferable that said zinc oxide have incorporated therein a minor proportion of an additive selected from the group consisting of aluminum oxide (Al<sub>2</sub>O<sub>3</sub>), iron oxide (Fe<sub>2</sub>O<sub>3</sub>), bismuth oxide (Bi<sub>2</sub>O<sub>3</sub>), magnesium oxide (MgO), calcium oxide (CaO), nickel oxide (NiO), cobalt oxide (CoO), niobium oxide (Nb<sub>2</sub>O<sub>5</sub>), tantalum oxide (Ta<sub>2</sub>O<sub>5</sub>), zirconium oxide (ZrO<sub>2</sub>), tungsten oxide (WO<sub>3</sub>), cadmium oxide (CdO), and chromium oxide (Cr<sub>2</sub>O<sub>3</sub>).

55 It has been discovered according to the invention that said sintered body 1 produces a superior non-linearity of the electrical characteristics when it is provided with silver electrodes prepared by applying silver paint to opposite surfaces thereof and firing at 100° C. to 850° C. in an oxidizing atmosphere such as air and oxygen. The n-value and C-value of so-produced non-linear resistors

vary with the compositions of the sintered body and electrodes, and their preparation method.

Since the non-linearity of the novel resistors is attributed to a non-ohmic contact between said sintered body 1 and electrodes 2 and 3, it is necessary for obtaining a desirable C-value and n-value to control the compositions of the sintered body 1 and the electrodes 2 and 3 and positions of the sintered body 1 and the electrodes 2 and 3.

It is necessary for achieving a low value of C of resultant non-linear resistors that the sintered body have an electrical resistivity less than 10 ohm-cm., said electrical resistivity being measured by a four point method in a per se conventional way.

Table 1 shows operable and optimal compositions of sintered body 1 for producing a non-linear resistor having an n-value higher than 3 and a high stability with temperature, humidity and electric load.

Table 2 shows operable and optimal compositions of silver electrodes 2 and 3 after heating for curing in order to produce the novel non-linear resistors in accordance with the invention.

Table 3 shows optimal combinations of sintered body 1 and silver electrodes 2, 3 for producing non-linear resistors having a C-value lower than 6 at a given current of 100 ma., an n-value higher than 4 and a high stability with temperature, humidity and electric load.

In the Tables 2 and 3, indicated in the specification, a sum of the weight percents of all ingredients should be 100 weight percent by controlling a weight percent of individual ingredient with operable or optimal weight percent indicated in the tables.

TABLE 1

| Operable Composition of Sintered Body (mol. percent) |                                                  | Optimal Composition of Sintered Body (mol. percent) |                                                  |
|------------------------------------------------------|--------------------------------------------------|-----------------------------------------------------|--------------------------------------------------|
| ZnO                                                  | Additive                                         | ZnO                                                 | Additive                                         |
| 100.....                                             | 0.....                                           | 99.9 to 98.0.....                                   | 0.1 to 2.0, Al <sub>2</sub> O <sub>3</sub> ..... |
| 99.95 to 90.0.....                                   | 0.05 to 10, Al <sub>2</sub> O <sub>3</sub> ..... | 99.9 to 98.0.....                                   | 0.1 to 2.0, Fe <sub>2</sub> O <sub>3</sub> ..... |
| 99.95 to 90.0.....                                   | 0.05 to 10, Fe <sub>2</sub> O <sub>3</sub> ..... | 99.9 to 98.0.....                                   | 0.1 to 2.0, Fe <sub>2</sub> O <sub>3</sub> ..... |
| 99.95 to 90.0.....                                   | 0.05 to 10, Bi <sub>2</sub> O <sub>3</sub> ..... | 99.9 to 98.0.....                                   | 0.1 to 2.0, Bi <sub>2</sub> O <sub>3</sub> ..... |
| 99.95 to 90.0.....                                   | 0.05 to 10, MgO.....                             | 99.9 to 98.0.....                                   | 0.1 to 2.0, MgO.....                             |
| 99.95 to 90.0.....                                   | 0.05 to 10, CaO.....                             | 99.9 to 98.0.....                                   | 0.1 to 2.0, CaO.....                             |
| 99.95 to 90.0.....                                   | 0.05 to 10, NiO.....                             | 99.9 to 98.0.....                                   | 0.1 to 2.0, NiO.....                             |
| 99.95 to 90.0.....                                   | 0.05 to 10, CoO.....                             |                                                     |                                                  |
| 99.95 to 90.0.....                                   | 0.05 to 10, Nb <sub>2</sub> O <sub>5</sub> ..... |                                                     |                                                  |
| 99.95 to 90.0.....                                   | 0.05 to 10, Ta <sub>2</sub> O <sub>5</sub> ..... |                                                     |                                                  |
| 99.95 to 90.0.....                                   | 0.05 to 10, ZrO <sub>2</sub> .....               |                                                     |                                                  |
| 99.95 to 90.0.....                                   | 0.05 to 10, WO <sub>3</sub> .....                |                                                     |                                                  |
| 99.95 to 90.0.....                                   | 0.05 to 10, CdO.....                             |                                                     |                                                  |
| 99.95 to 90.0.....                                   | 0.05 to 10, Cr <sub>2</sub> O <sub>3</sub> ..... |                                                     |                                                  |

TABLE 2  
[Operable Composition of Electrode, Wt. Percent]

| Ag                                              | PbO             | SiO <sub>2</sub> | B <sub>2</sub> O <sub>3</sub> | Bi <sub>2</sub> O <sub>3</sub> | CdO           | CuO           |
|-------------------------------------------------|-----------------|------------------|-------------------------------|--------------------------------|---------------|---------------|
| 100.....                                        |                 |                  |                               |                                |               |               |
| 70 to 99.5.....                                 | 0.25 to 27..... | 0.02 to 15.....  | 0.01 to 15.....               | 0 to 6.0.....                  | 0 to 6.0..... | 0 to 6.0..... |
| [Optimal Composition of Electrode, Wt. Percent] |                 |                  |                               |                                |               |               |
| 80 to 98.....                                   | 1.2 to 17.....  | 0.1 to 6.0.....  | 0.06 to 6.0.....              | 0 to 2.0.....                  | 0 to 2.0..... | 0 to 2.0..... |

TABLE 3.—OPTIMAL COMBINATIONS OF SINTERED BODY AND ELECTRODE

| Composition of Sintered Body (Mol. Percent) |                                                  | Composition of Electrode (Wt. Percent) |                |                  |                               |                                |               |               |
|---------------------------------------------|--------------------------------------------------|----------------------------------------|----------------|------------------|-------------------------------|--------------------------------|---------------|---------------|
| ZnO                                         | Additive                                         | Ag                                     | PbO            | SiO <sub>2</sub> | B <sub>2</sub> O <sub>3</sub> | Bi <sub>2</sub> O <sub>3</sub> | CdO           | CuO           |
| 99.9 to 98.....                             | 0.1 to 2.0, Fe <sub>2</sub> O <sub>3</sub> ..... | 80 to 98.....                          | 1.2 to 17..... | 0.1 to 6.0.....  | 0.06 to 6.0.....              | 0 to 2.0.....                  | 0 to 2.0..... | 0 to 2.0..... |

The sintered body 1 can be prepared by a per se well known ceramic technique. The starting materials in the compositions defined in Table 1 are mixed in a wet mill so as to produce homogeneous mixtures. The mixtures are dried and pressed in a mold into desired shapes at a pressure from 100 kg./cm.<sup>2</sup> to 1000 kg./cm.<sup>2</sup>. The pressed bodies are sintered in air at 1250° C. to 1450° C. for 1 to 3 hours, and then furnace-cooled to room temperature (about 15° to about 30° C.). The pressed bodies are preferably sintered in non-oxidizing atmosphere such as

nitrogen and argon when it is desired to reduce the electrical resistivity. The electrical resistivity also can be reduced by air-quenching from the sintering temperature to room temperature even when the pressed bodies are fired in air.

5 The mixtures may be preliminarily calcined at 700 to 1000° C. and pulverized for easy fabrication in the subsequent pressing step. The mixture to be pressed may be admixed with a suitable binder such as water, polyvinyl alcohol, etc.

10 It is advantageous that the sintered body be lapped at the opposed surfaces by abrasive powder such as silicon carbide in a particle size of 300 meshes to 1500 meshes.

15 The sintered bodies are coated at the opposed surfaces thereof by a silver electrode paint in a per se conventional manner such as by a spray method, screen printing method or brushing method. It is necessary that the silver electrode paint have a solid ingredient composition as defined in Tables 2 and 3 after it is fired at 100° C. to 850° C. in air. Solid ingredients having compositions defined in Tables 2 and 3 can be prepared in a per se conventional manner by mixing commercially available powders with organic resin such as epoxy, vinyl and phenol 20 25 resin in an organic solvent such as butyl acetate, toluene or the like so as to produce silver electrode paints.

25 The silver powder may be in the form of metallic silver, or in the form of silver carbonate or silver oxide, or in any other form which in firing at the temperatures 30 employed will be converted to metallic silver. Therefore, the term "silver" as used throughout this specification and the claims appended hereto in connection with the silver composition before it is fired, is meant to include silver in any form which in firing will be converted to metallic silver. The viscosity of the resultant silver electrode paints can be controlled by the amounts of resin and solvent. Particle size of solid ingredients also are required to be controlled in the range of 0.1 $\mu$  to 5 $\mu$ .

35 40 Lead wires can be applied to the silver electrodes in a per se conventional manner by using conventional solder having a low melting point. It is convenient to employ a conductive adhesive comprising silver powder and resin in an organic solvent for connecting the lead wires to the silver electrodes.

45 Non-linear resistors according to this invention have a high stability to temperature and in the load life test, which is carried out at 70° C. at a rating power for 500 hours. The n-value and C-value do not change remark-

ably after heating cycles and load life test. It is preferable for achieving a high stability to humidity that the resultant non-linear resistors are embedded in a humidity proof resin such as epoxy resin and phenol resin in a per se well known manner.

70 According to the invention, it has been discovered that the curing method of the applied silver electrode paint has a great effect on the n-value of the resultant non-linear resistors. The n-value will not be optimal when 75 the applied silver electrode paint is heated in a non-oxidiz-

ing atmosphere such as nitrogen and hydrogen for curing. It is necessary for obtaining a high *n*-value that the applied silver electrode paint be cured by heating in an oxidizing atmosphere such as air and oxygen.

Silver electrodes prepared by any other method than by silver painting result in a poor *n*-value. For example, the sintered body does not produce a non-linear resistor when it is provided with silver electrodes at the opposite surfaces by electroless plating or electrolytic plating in conventional manner. Silver electrodes prepared by vacuum evaporation or chemical deposition result in an *n*-value less than 3.

The following examples are given as illustrative of the presently-preferred method of proceeding according to the present invention; however, it is not intended that the scope of said invention be limited to the specific examples.

#### EXAMPLE 1

Starting material according to Table 4 is mixed in a wet mill for 5 hours.

The mixture is dried and pressed in a mold into a disc of 13 mm. in diameter and 2.5 mm. in thickness at the pressure of 340 kg./cm.<sup>2</sup>.

The pressed body is sintered in air at 1350° C. for 1 hour, and then quenched to room temperature (about 15° to about 30° C.). The sintered disc is lapped at the opposite surfaces thereof by silicon carbide in a particle size of 600 meshes. Resulting sintered disc has a size of 10 mm. in diameter and 1.5 mm. in thickness. The sintered disc is coated at the opposite surfaces thereof with a silver electrode paint by a conventional brushing method. The silver electrode paint employed has the solid ingredient composition according to Table 5 and is prepared by mixing with vinyl resin in amyl acetate. The coated disc is fired at 500° C. for 30 minutes in air.

Lead wires are attached to the silver electrodes by means of silver paint. The electric characteristics of the resultant resistor and of other similarly prepared resistors are shown in Table 4.

TABLE 5.—COMPOSITION OF SILVER ELECTRODE (WT. PERCENT)

| Ag | PbO | SiO <sub>2</sub> | B <sub>2</sub> O <sub>3</sub> | CdO |
|----|-----|------------------|-------------------------------|-----|
| 90 | 7.0 | 2.0              | 0.7                           | 0.3 |

TABLE 4

| Starting Materials (mol. percent) | Additives                            | Electric Characteristics of Resultant Resistors |          | <i>n</i> |
|-----------------------------------|--------------------------------------|-------------------------------------------------|----------|----------|
|                                   |                                      | C (at a given current of 100 m a.)              | <i>n</i> |          |
| 100                               | 0                                    | 12.4                                            | 3.24     |          |
| 99.5                              | 0.5, Al <sub>2</sub> O <sub>3</sub>  | 1.67                                            | 3.59     |          |
| 98.5                              | 1.5, Al <sub>2</sub> O <sub>3</sub>  | 1.71                                            | 3.40     |          |
| 99.95                             | 0.05, Fe <sub>2</sub> O <sub>3</sub> | 2.77                                            | 3.30     |          |
| 99.9                              | 0.1, Fe <sub>2</sub> O <sub>3</sub>  | 2.59                                            | 4.02     |          |
| 99.8                              | 0.2, Fe <sub>2</sub> O <sub>3</sub>  | 1.73                                            | 4.32     |          |
| 99.5                              | 0.5, Fe <sub>2</sub> O <sub>3</sub>  | 1.56                                            | 4.83     |          |
| 99.0                              | 1.0, Fe <sub>2</sub> O <sub>3</sub>  | 1.90                                            | 4.28     |          |
| 98.0                              | 2.0, Fe <sub>2</sub> O <sub>3</sub>  | 2.45                                            | 4.05     |          |
| 95.0                              | 5.0, Fe <sub>2</sub> O <sub>3</sub>  | 4.50                                            | 3.25     |          |
| 90.0                              | 10.0, Fe <sub>2</sub> O <sub>3</sub> | 10.5                                            | 3.10     |          |
| 99.5                              | 0.5, Bi <sub>2</sub> O <sub>3</sub>  | 1.91                                            | 3.61     |          |
| 99.0                              | 1.0, MgO                             | 4.21                                            | 4.24     |          |
| 99.0                              | 1.0, CaO                             | 3.85                                            | 3.90     |          |
| 99.0                              | 1.0, NiO                             | 2.99                                            | 4.11     |          |
| 99.0                              | 1.0, CoO                             | 2.58                                            | 3.88     |          |
| 99.5                              | 0.5, Nb <sub>2</sub> O <sub>5</sub>  | 2.56                                            | 3.68     |          |
| 99.5                              | 0.5, Ta <sub>2</sub> O <sub>5</sub>  | 2.84                                            | 3.69     |          |
| 99.0                              | 1.0, ZrO <sub>2</sub>                | 3.67                                            | 3.91     |          |
| 99.0                              | 1.0, WO <sub>3</sub>                 | 2.15                                            | 3.52     |          |
| 99.0                              | 1.0, CdO                             | 2.11                                            | 3.16     |          |
| 99.5                              | 0.5, Cr <sub>2</sub> O <sub>3</sub>  | 3.49                                            | 3.69     |          |

#### EXAMPLE 2

A sintered disc in a composition of 99.5 mol. percent of zinc oxide and 0.5 mol. percent of iron oxide is pre-

pared in the same manner as that in Example 1. The sintered disc has a size of 10 mm. in diameter and 1.5 mm. in thickness after lapping. Various silver electrode paints are applied to the opposite surfaces of the sintered disc and fired at 500° C. for 30 minutes in air. The silver electrode paints have solid ingredient compositions shown in Table 6 and are prepared by mixing 100 weight parts of said solid ingredient compositions with 1 to 20 weight parts of epoxy resin in 20 to 40 weight parts of butyl alcohol. The resultant non-linear resistors exhibit desirable C-values and *n*-values as indicated in Table 6. It will be readily understood that the electrode compositions have a great effect on the electrical characteristics of the resultant non-linear resistors.

#### EXAMPLE 3

The resistors of Example 1 are tested according to the methods used in the electronic component parts. The load life test is carried out at 70° C. ambient temperature at 1 watt rating power for 500 hours. The heating cycle test is carried out by repeating 5 times the cycle in which said resistors are kept at 85° C. ambient temperature for 30 minutes, cooled rapidly to -20° C. and then kept at such temperature for 30 minutes. After heating cycles and load life test, the C-value and *n*-value do not change more than 5% and 10%, respectively.

TABLE 6

| Composition of Electrode (wt. percent) |      |                  |                               |                                |     | The Characteristics of the Resultant Resistors |          |     |
|----------------------------------------|------|------------------|-------------------------------|--------------------------------|-----|------------------------------------------------|----------|-----|
| Ag                                     | PbO  | SiO <sub>2</sub> | B <sub>2</sub> O <sub>3</sub> | Bi <sub>2</sub> O <sub>3</sub> | CdO | C (at a given current of 100 ma.)              | <i>n</i> |     |
| 100                                    |      |                  |                               |                                |     | 0.95                                           | 3.3      |     |
| 95                                     | 3.5  | 1.0              | 0.5                           |                                |     | 1.10                                           | 4.2      |     |
| 95                                     | 3.3  | 0.8              | 0.3                           | 0.6                            |     | 1.12                                           | 4.5      |     |
| 90                                     | 6.2  | 2.0              | 0.8                           | 1.0                            |     | 1.25                                           | 4.5      |     |
| 90                                     | 6.5  | 2.0              | 0.8                           |                                | 0.7 | 1.26                                           | 4.8      |     |
| 90                                     | 6.5  | 2.0              | 0.8                           |                                |     | 1.54                                           | 5.2      |     |
| 90                                     | 6.5  | 2.0              | 0.8                           |                                | 0.4 | 1.32                                           | 4.8      |     |
| 85                                     | 10.0 | 3.0              | 1.0                           | 0.3                            | 0.4 | 0.3                                            | 2.37     | 4.5 |
| 75                                     | 14.0 | 5.0              | 2.0                           | 3.0                            | 0.6 | 0.4                                            | 3.26     | 3.5 |

What is claimed is:

1. A non-linear resistor comprising a sintered wafer consisting essentially of zinc oxide, and silver paint electrodes applied to opposite surfaces of said sintered wafer, said electrodes consisting essentially of fired silver paint.
2. A non-linear resistor according to claim 1, wherein said sintered wafer comprises 99.95 to 90 mol. percent of zinc oxide (ZnO) and 0.05 to 10.0 mol. percent of at least one oxide selected from the group consisting of iron oxide (Fe<sub>2</sub>O<sub>3</sub>), aluminum oxide (Al<sub>2</sub>O<sub>3</sub>), bismuth oxide (Bi<sub>2</sub>O<sub>3</sub>), magnesium oxide (MgO), calcium oxide (CaO), nickel oxide (NiO), cobalt oxide (CoO), niobium oxide (Nb<sub>2</sub>O<sub>5</sub>), tantalum oxide (Ta<sub>2</sub>O<sub>5</sub>), zirconium oxide (ZrO<sub>2</sub>), tungsten oxide (WO<sub>3</sub>), cadmium oxide (CdO), and chromium oxide (Cr<sub>2</sub>O<sub>3</sub>).
3. A non-linear resistor according to claim 1, wherein said sintered wafer comprises 99.9 to 98.0 mol. percent of zinc oxide (ZnO) and 0.1 to 2.0 mol. percent of at least one oxide selected from the group consisting of aluminum oxide (Al<sub>2</sub>O<sub>3</sub>), iron oxide (Fe<sub>2</sub>O<sub>3</sub>), bismuth oxide (Bi<sub>2</sub>O<sub>3</sub>), magnesium oxide (MgO), calcium oxide (CaO) and nickel oxide (NiO).
4. A non-linear resistor according to claim 2, wherein said silver electrodes have a composition of 100 wt. percent of silver.
5. A non-linear resistor according to claim 1, wherein said silver electrodes have the composition comprising 70 to 99.5 wt. percent of silver, 0.25 to 27 wt. percent of lead oxide (PbO), 0.02 to 15 wt. percent of silicon dioxide

( $\text{SiO}_2$ ), 0.01 to 15 wt. percent of boron trioxide ( $\text{B}_2\text{O}_3$ ), 0 to 6.0 wt. percent of bismuth oxide ( $\text{Bi}_2\text{O}_3$ ), 0 to 6.0 wt. percent of cadmium oxide ( $\text{CdO}$ ) and 0 to 6.0 wt. percent of cupric oxide ( $\text{CuO}$ ).

6. A non-linear resistor according to claim 1, wherein said silver electrodes have the composition comprising 80 to 98 wt. percent of silver, 1.2 to 17 wt. percent of lead oxide ( $\text{PbO}$ ), 0.1 to 6.0 wt. percent of silicon dioxide ( $\text{SiO}_2$ ), 0.06 to 6.0 wt. percent of boron trioxide ( $\text{B}_2\text{O}_3$ ), 0 to 2.0 wt. percent of bismuth oxide ( $\text{Bi}_2\text{O}_3$ ), 0 to 2.0 wt. percent of cadmium oxide ( $\text{CdO}$ ) and 0 to 2.0 wt. percent cupric oxide ( $\text{CuO}$ ).

7. A non-linear resistor according to claim 1, wherein said sintered wafer comprises 99.9 to 98.0 mol. percent of zinc oxide ( $\text{ZnO}$ ) and 0.1 to 2.0 mol. percent of iron oxide ( $\text{Fe}_2\text{O}_3$ ), and said silver electrodes have the composition comprising 80 to 98 wt. percent of silver, 1.2 to 17 wt. percent of lead oxide ( $\text{PbO}$ ), 0.1 to 6.0 wt. percent of silicon dioxide ( $\text{SiO}_2$ ), 0.06 to 6.0 wt. percent of boron trioxide ( $\text{B}_2\text{O}_3$ ), 0 to 2.0 wt. percent of bismuth oxide ( $\text{Bi}_2\text{O}_3$ ), 0 to 2.0 wt. percent of cadmium oxide ( $\text{CdO}$ ) and 0 to 2.0 wt. percent of cupric oxide ( $\text{CuO}$ ).

## References Cited

## UNITED STATES PATENTS

|           |         |               |       |           |
|-----------|---------|---------------|-------|-----------|
| 2,786,819 | 3/1957  | Smith et al.  | ----- | 338—22    |
| 2,977,558 | 3/1961  | Hampton       | ----- | 338—22    |
| 3,037,942 | 6/1962  | Ingold et al. | ----- | 252—518 X |
| 3,075,122 | 1/1963  | Lehmann       | ----- | 252—518 X |
| 3,219,480 | 11/1965 | Girard        | ----- | 338—22 X  |
| 3,264,229 | 8/1966  | Klein         | ----- | 252—518   |
| 1,822,742 | 9/1931  | McEachron     | ----- | 338—21    |
| 2,027,277 | 1/1936  | Habann        | ----- | 338—20    |

## FOREIGN PATENTS

|         |         |                |
|---------|---------|----------------|
| 479,580 | 12/1951 | Canada.        |
| 618,966 | 3/1949  | Great Britain. |

## 15 OTHER REFERENCES

"Zinc Oxide Rediscovered," New Jersey Zinc Co., 1957, TP 245 Z7N4, pp. 28, 29, 30, 31, 32, 33, 34.

20 REUBEN EPSTEIN, Primary Examiner

U.S. Cl. X.R.

29—612, 621; 338—22, 327